

Jan. 9, 1934.

E. O. RHODES

1,942,980

PROCESS OF COOKING LIQUID OR LIQUEFIABLE BITUMINOUS MATERIAL

Filed Dec. 6, 1930

3 Sheets-Sheet 1



Jan. 9, 1934.

E. O. RHODES

1,942,980

PROCESS OF COKING LIQUID OR LIQUEFIABLE BITUMINOUS MATERIAL

Filed Dec. 6, 1930

3 Sheets-Sheet 2



Fig. 2

INVENTOR.  
*Edmund O. Rhodes.*  
BY  
*Jesse R. Langley*  
ATTORNEY.

Jan. 9, 1934.

E. O. RHODES

1,942,980

PROCESS OF COKING LIQUID OR LIQUEFIABLE BITUMINOUS MATERIAL

Filed Dec. 6, 1930

3 Sheets-Sheet 3



Fig. 3

INVENTOR.  
*Edmund O. Rhodes.*  
BY  
*Jesse R. Langley* ATTORNEY.

## UNITED STATES PATENT OFFICE

1,942,980

## PROCESS OF COKING LIQUID OR LIQUEFIABLE BITUMINOUS MATERIAL

Edmund O. Rhodes, Pittsburgh, Pa., assignor to  
American Tar Products Co., Inc., a corporation  
of Delaware

Application December 6, 1930. Serial No. 500,540

4 Claims. (Cl. 202—32)

This invention relates to a process of treating bituminous materials and more particularly to an improved process of producing coke therefrom.

5 In an application of Edmund O. Rhodes, Serial No. 338,644, filed February 9, 1929, a process is described in which liquid or liquefiable bituminous material is introduced into a highly-heated retort preferably with steam or other gas, and 10 coked. The present invention is directed to improvements in the manner of introducing fluid or liquefiable bituminous material into a coking chamber and in the manner of producing coke therein. The feeding of the material into the 15 coking chamber is so conducted that the difficulties usually encountered in coking fluid bituminous materials, are practically eliminated.

In accordance with the present invention fluid bituminous material is introduced into a highly heated chamber preferably by means of a spray and preferably with steam. Other gases such as carbon dioxide, carbon monoxide, hydrogen, methane and nitrogen or mixtures of the same, including flue gases, or the gaseous products of combustion from gaseous, liquid or solid fuels, or those produced by the carbonization of coal, may be used for this purpose but steam is preferred.

Conditions for coking may be further improved by having present in the coking chamber a supply of gases introduced if desired, by means other than through the sprays for atomizing the bituminous material. The gases may be steam or any of those mentioned above or mixtures of the same including hot combustion gases or coke oven gases. These gases may be passed through the chamber in any direction and a fresh supply continuously provided while the bituminous material is being introduced and during the coking period or early stages thereof.

The gases employed should preferably contain substantially no free oxygen. Air, for instance, should be excluded as much as is normally possible during the charging or coking operations.

The fluid bituminous material under certain conditions may be heated to any desired temperature before feeding it into the coking chamber. It is, in certain cases, advantageous to heat the material under pressure and feed it into a coking chamber at a lower pressure.

Extremely good results are obtained, in any case, by controlling the rate of feeding the fluid material into the coking chamber. In general, it may be said that the most satisfactory rate is such that fluid bituminous material is converted to a substantially semi-cooked or to a partially

coked but yet fluid or plastic condition while falling in the chamber.

The resulting material is accumulated in this plastic condition in a shallow body in the coking chamber to permit coalescence. Further bituminous material of such plastic consistency is gradually added to the said body while at the same time proceeding with the coking operation.

The rate of feeding the fluid bituminous material depends largely on the temperature and pressure of the coking chamber and of the material being fed. It depends also on the nature of the bituminous matter. A crude tar would be fed in at a lower rate under given conditions than a hard pitch for instance. It is desirable that the rate in each case be such that while the material is dropping through free space in the coking chamber, a portion of the volatile matter therein is removed before it reaches the bottom of its fall. By such operation enough volatile matter is left so that particles of the material coalesce before complete coking takes place.

The introduction of bituminous material is stopped when the coking chamber is charged to the desired level. The coking operation is continued until the material therein is converted into a dry or substantially dry coke, after which it is removed and the charging operation repeated.

Coke of excellent structure may be produced by the present process from such materials as coal tars including coke oven tar; oil tars from water-gas and oil-gas manufacturing plants; petroleum oils; pitches or residua from the aforesaid materials; and mixtures of these substances.

Examples of apparatus which may be employed in the process of the present invention are shown in the accompanying drawings in which,

Figure 1 is a vertical sectional view of means for preheating liquid bituminous matter, and of a coking retort oven combined with the said heating means;

Fig. 2 is a view in enlarged vertical section of means for introducing liquid bituminous material simultaneously with steam or other gas into a coking retort oven;

Fig. 3 is a vertical sectional view taken longitudinally of a coking retort oven including means for producing a current of gas therethrough; and

Figure 4 is a fragmentary vertical sectional view taken transversely of a coke oven chamber and showing heating flues in the side walls of the said chamber.

In the apparatus shown in Fig. 1, bituminous

60

65

70

75

80

85

90

95

105

100

110

material such as pitch, or tar which has been preferably previously dehydrated, are forced under pressure through a heated bank of tubes 1 by means of a pump 2 and sprayed into a heated coking chamber 3 which is under a lower pressure, for example, substantially atmospheric pressure. A bank of tubes, such as tubes 1, is preferable for heating the material although good results may be obtained by substituting a still and 10 pumping tar or pitch from the still to the coking chamber.

Fluid bituminous material may also be fed from a tank car or other container with or without preheating. When the preheater is not in use, 15 valves 4 and 5 are closed and material is fed through pipes 6 and 7 to the sprays 8 the valve 9 being open. When material is fed through the preheater, the valves 4 and 9 are closed and the valve 5 is open. By opening the 20 valves 4 and 9 and closing the valve 5, the material may be by-passed to a vapor release box (not shown) and the unvaporized material conveyed through the pipes 6 and 7 to the sprays 8.

Although the chamber 3 may be any suitable 25 type of coking retort which may be heated to the desired temperature preferably by applying the heating medium to substantially its entire outer surface, I have shown, for purposes of illustration, the ordinary type of by-product oven used 30 for coking coal and usually arranged in batteries comprising a plurality of such ovens as described, for example, in U. S. Patent No. 1,374,546 of Joseph Becker, dated April 12, 1921. These ovens are built of refractory material, such as 35 silica bricks or the like, and the present process is particularly adapted to their use.

Heating flues 3' are provided in the side walls of the oven chamber shown. These flues extend substantially through the entire height of the 40 walls.

The spraying means 8 are directed downwardly through the openings in the top of the oven. Valves 10 control the passage of bituminous liquid material through the sprays 8 and 45 also permit the use of steam or other gas from a pipe line 11 for aiding the introduction of the bituminous liquid material into the chamber 3.

The valves 10 are illustrated in detail in Fig. 2. Each valve 10 is provided with a spray 8 extending down to the coking retort oven 3 through a charging hole 12 and through a suitable opening 50 13 in the charging hole cover 14, the opening 13 being luted with fireclay as shown.

The spray 8 is provided with an extension 15 passing into the interior of the valve-chamber 10 and terminating in a valve seat 16, the flow of bituminous material through the extension 15 being regulated by varying the distance between the 55 valve seat 16 and a corresponding valve member 17.

The valve member 17 is conveniently carried by a hollow spindle 18 which extends into the interior of the extension 15 and which also passes through a gland 19 and communicates through a valve 20 with the line 11 supplying steam or other gas. By means of a handwheel 21, the spindle 18 and the valve member 17 may be raised or lowered, thus opening or closing the orifice through which bituminous liquid material discharges from the line 7 through the offtake 8 into the coke oven 2.

A handwheel 22 is provided and engages the extension 15 and spray 8 by rotation of which connection between these two may be severed. 75 The spray 8 may be thereby withdrawn from the

charging hole 12 by means of a suitable handle 23.

The lower end 24 of the offtake 8 is preferably so shaped that little or none of the bituminous material treated will be sprayed onto the walls of the coking chamber. When the process is carried on in a by-product oven of the long and narrow type, as in case of the usual horizontal oven, the end 24 may be of the shape shown. That is, it may be provided with a flare, as shown, having a relatively long and narrow opening co-axially disposed with the longitudinal axis of the coking retort oven.

The oven is provided with a suitable vapor outlet which may be in the form of the usual standpipe 25. The vapors pass into a collecting main 90 26 and are condensed.

In the apparatus shown in Fig. 3, means are provided for passing gases through the oven 3 while spraying bituminous material into the oven by means of the sprays 8. For this purpose a pipe 27 is connected to an opening 28 at the end of the coke oven 3 opposite to the end at which the standpipe 25 is placed. In this way the gases fed into the oven through pipe 27 pass through the sprays of bituminous material and carry with them any vaporized matter as they pass through the standpipe 25.

For the purpose of feeding fluid bituminous material to the oven, the sprays 8 may be connected to a loop 29. The fluid bituminous material may 105 be fed continuously through this loop which may conduct the material from any source and back again. The piping in the loop 29 is shown in an inclined position to provide for drainage of the bituminous material back to its source when the 110 loop is not in use.

When charging with tar, either crude or dehydrated, it may, if desired, be preheated to substantially 700° F. and fed under super-atmospheric pressure. The coking chamber for most 115 purposes is heated to a temperature above 1000° F. and preferably from substantially 1400° F. to 2200° F.

In order that the coke produced may be easily pushed out, it is necessary to obtain a proper coke structure. This is particularly true with respect to the coke lying adjacent the bottom of the chamber. This coke should be quite dense and firm, because if a layer of granular coke of appreciable depth is formed the pushing operation 125 is rendered quite difficult. When charging the coking chamber, therefore, it is advantageous to feed the material rapidly at first after which the rate of feed may be varied if desired. In certain cases it may be desirable to decrease the rate of 130 feed substantially, after which the rate may be maintained substantially constant or gradually reduced until the charging is completed.

To insure the formation of a proper coke structure at the bottom of a coking chamber, it has 135 been found that the rate of feed can be initially quite high even to the extent that tar or pitch in a substantially free-flowing condition, collects on the bottom of the coking chamber at the beginning of the charging period. For example, this 140 precaution may be taken until the material in the oven has reached a substantial depth of for instance one foot more or less, assuming that the oven is about 40 feet long, 10 feet high and 16 inches wide and the height of the coke produced 145 in the oven is 4 to 6 feet.

The following examples are given to illustrate the process of the present invention:

*Example 1.*—The special charging hole covers are put in place and sealed and the sprays di- 150

rected downwardly into the charging holes in a by-product oven. Steam is turned into the sprays and adjusted to about 10 pounds pressure per square inch. Pitch having a melting point of 5 about 260° F. is then admitted to the sprays with the steam at an average rate of about 885 gallons per hour for about 2½ hours, after which the sprays are removed and the usual charging hole covers put in place. The coking is continued 10 for about 4½ hours in which time the coke formed has properly shrunk.

In the above example, the temperature of the oven wall at the start is about 1825° F. and at the finish about 1895° F.

15 *Example 2.*—Pitch having a melting point of about 280° F. is charged without steam into a by-product oven at the average rate of 920 gallons per hour for about 2¼ hours and the coking completed in about 5½ hours. The temperature of 20 the oven wall before charging is about 1760° F. and after pushing out the finished coke the temperature is about 1920° F.

The current required in each of the above cases to start the pushing machine when applied to the 25 coke is about 120 amperes and about 100 amperes after the coke is set in motion.

It has been found in the process of the present invention that the presence of steam or other gaseous substances during the charging and coking operations prevents the breaking down of the 30 bituminous vapors, particularly in carbon. It is believed that this may be explained in the following way: Assume that the walls of the coking chamber are heated to a temperature of, say, 35 1800° F. and that liquefied high melting point pitch for instance is sprayed into the coking chamber at a rate of, say, 400 gallons per hour. Under these conditions it has been found that the vapors that are distilled from the pitch break 40 down to form a considerable amount of carbon in the form of lampblack which leaves the coking chamber with the vapors.

If under these conditions steam or other gaseous substances are introduced into the coking 45 chamber, either with the pitch or separately, the formation of lampblack may be diminished or even entirely eliminated. It is believed that the steam or other gaseous substances accomplish this result by absorbing part of the heat from 50 the coking chamber that otherwise would be transmitted to the bituminous vapors. In this way the steam or other gaseous substances may be considered as inert materials that exert a cooling effect on the vapors or prevent the super- 55 heating of the vapors by absorbing a part of the total available heat.

This is further substantiated by the fact that if the substance to be coked is charged more rapidly into the coking chamber it is apparently 60 not necessary to employ any steam or other gaseous substances to prevent lampblack formation. To illustrate this point let us assume that the coking chamber mentioned above with wall temperatures of say 1800° F. is being charged with 65 liquid high melting point pitch at the rate of 400 gallons per hour and that lampblack formation is taking place due to an excessive decomposition of the pitch vapors. If, at such time, steam or other gaseous substances are introduced into the 70 coking chamber the decomposition of the vapors will be lessened or eliminated with consequent reduction or elimination of lampblack formation.

On the other hand, it has been found that if the rate of charging is increased from, say, 400 gallons 75 per hour to, say, 800 or 1000 gallons per hour the

lampblack formation will again be reduced or eliminated for the reason that the higher pitch feed has caused the evolution of a greater quantity of vapors which cannot be superheated to the same extent as the smaller amount of vapor originally present with the same amount of total available heat and a lower rate of charging. Furthermore, with the higher rate of feed the vapors are evolved so rapidly that they are forced out of the coking chamber and therefore subjected to the high temperatures for only a comparatively short time.

In other words, it has been found that when liquid bituminous material is coked the effect produced by the presence of steam or other gas may be obtained by introducing the material into the coking chamber at the proper rate, that is, at such a rate that large volumes of vapors are formed and yet at such rate that the material deposited in the chamber is of the proper consistency for forming coke of the desired texture.

It has been found that the use of steam or other gas, or the employment of a proper rate of feed that will produce similar results, or the employment of a combination of these two methods constitute a very important part of this process. A coking chamber lined with a refractory material, such as silica brick, is most efficiently operated at rather high temperatures, say above 1600° F. If operated at low temperatures, or if operated in such manner that the walls are chilled to low temperatures the life of the walls is considerably shortened by the formation of cracks and the disintegration of the brick.

It has been found that by the employment of steam or other gas or a suitable rate of charging or a combination of the two, high wall temperatures may be employed so that disintegration of the refractory walls is avoided; lampblack formation, due to excessive decomposition of the vapors, may be prevented, and coke of good structure may be produced. These factors, it is believed, determine the success of this method of coking fluid bituminous materials.

The difficulties accompanying the heating of tar or pitch to carbonize the same are well known. In the present process, coke is produced directly from liquid bituminous materials without the difficulties and dangers usually resulting therefrom. There is no trouble from foaming, substantially no formation of lampblack or wall carbon, and substantially no burning of bituminous material within the oven.

The coke produced in the manner described is of such texture that when produced in for instance a by-product coke oven such as that described above, it may be pushed out in the convenient manner that coke from coal is pushed out. There is no spalling of the brick lining, or sticking of the coke, and consequently no destruction of the brick lining. The coke is comparatively free from ash and is in strong block-like form substantially free from powder and from an excessive amount of so-called fingering.

I claim as my invention:

1. A process of manufacturing coke from bituminous material selected from a group consisting of liquid bituminous material and liquefiable bituminous material in an externally heated by-product oven having side walls with heating flues extending substantially through the entire height of the walls, which process comprises heating the side walls of the oven to maintain the coking chamber at coking temperature, charging the bituminous material in a free-

flowing condition into the oven, maintaining the oven above the level of material deposited therein substantially completely filled with vapors from the said bituminous material and at the same time preventing excessive foaming, the said charging being conducted at a rate that effects the emission of vapors from the oven at a greater rate than that at which vapors evolved are superheated and decomposed to a substantial extent during their passage through the oven, thereby reducing decomposition and formation of lampblack; withdrawing vapors from the oven; collecting the resulting residual material in the oven while simultaneously coking it, continuing the coking of the accumulated material to devolatilize and shrink the coked material, and removing coke from the oven by a pushing operation.

2. A process of manufacturing coke from bituminous material selected from a group consisting of liquid bituminous material and liquefiable bituminous material in an externally heated by-product oven having side walls with heating flues extending substantially through the entire height of the walls, which process comprises heating the side walls of the oven to maintain the coking chamber at coking temperature, charging the bituminous material in a free-flowing condition into the oven, separately passing a gaseous medium substantially free from uncombined oxygen through the oven while charging said bituminous material into said oven, the said gaseous medium upon introduction into the oven being at a lower temperature than the temperature of the coke oven, maintaining in the coke oven during the charging period a mixture of said gaseous medium with vapors from the said bituminous material to prevent superheating and decomposition of the vapors to a substantial extent, withdrawing vapors and gases from the oven, collecting the resulting residual material in the oven while simultaneously coking it, continuing the coking of the accumulated material to devolatilize and shrink the coked material, and removing coke from the oven by a pushing operation.

3. A process of manufacturing coke from bituminous material selected from a group consisting of liquid bituminous material and liquefiable bituminous material in an externally heat-

ed by-product oven having side walls with heating flues extending substantially through the entire height of the walls, which process comprises heating the side walls of the oven to maintain the coking chamber at coking temperature, charging the bituminous material in a free-flowing condition into the oven, maintaining the oven above the level of material deposited therein substantially completely filled with vapors from the said bituminous material and at the same time preventing excessive foaming, varying the rate of said charging but introducing the bituminous material during the charging thereof at a rate that effects the emission of vapors from the oven at a greater rate than that at which vapors evolved are superheated and decomposed to a substantial extent during their passage through the oven, thereby reducing decomposition and formation of lampblack; withdrawing vapors from the oven; collecting the resulting residual material in the oven while simultaneously coking it, continuing the coking of the accumulated material to devolatilize and shrink the coked material, and removing coke from the oven by a pushing operation.

4. A process of manufacturing coke from pitch in an externally heated by-product oven having side walls with heating flues extending substantially through the entire height of the walls, which process comprises heating the side walls of the oven to maintain the coking chamber at coking temperature, charging the pitch in a free-flowing condition into the oven, maintaining the oven above the level of material deposited therein substantially completely filled with vapors from the said pitch and at the same time preventing excessive foaming, the said charging being conducted at a rate that effects the emission of vapors from the oven at a greater rate than that at which vapors evolved are superheated and decomposed to a substantial extent during their passage through the oven, thereby reducing decomposition and formation of lampblack; withdrawing vapors from the oven; collecting the resulting residual material in the oven while simultaneously coking it, continuing the coking of the accumulated material to devolatilize and shrink the coked material, and removing coke from the oven by a pushing operation.

EDMUND O. RHODES.

125

130

135

140

145

150

85

90

95

100

105

110

115

120

125